

FIP8309 OR 2,231,426  
UNION OF BELGIUM & IRELAND

111 Patented Feb. 11, 1941

2,231,426

## UNITED STATES PATENT OFFICE

2,231,426

## METHOD OF BLEACHING GRAY GOODS

Hans O. Kauffmann, Eggertsville, N. Y., assignor  
to Buffalo Electro-Chemical Company, Inc.,  
Buffalo, N. Y.No Drawing. Application May 10, 1939,  
Serial No. 272,915

9 Claims. (Cl. 8—111)

The present invention relates to a method for bleaching cellulose, whether natural or regenerated, particularly in the form of fibers and filaments. More particularly it relates to a method 5 for bleaching such fibers and filaments with alkaline solutions containing hydrogen peroxide, or material generating hydrogen peroxide, by first subjecting the cellulose to the alkaline bleaching solution under conditions where a low liquor ratio 10 is maintained, and then subjecting the cellulose to an alkaline bleach where a relatively high liquor ratio is maintained.

Heretofore it has been suggested that cellulose be bleached by dampening the fibers with peroxide bleaching solutions and permitting the 15 fibers to bleach in the dampened condition. Relatively high concentrations of hydrogen peroxide are required to produce goods of excellent white and considerable bleaching agent remains at the 20 termination of the bleaching period. In general, bleaching in the damp condition with this type of solution is effected at room temperatures or slightly elevated temperatures. Although considerable energy is saved, the peroxide consumption 25 is high.

It has also been proposed to bleach cellulose in order to obtain excellent white by heating the fibers in a considerable body of bleaching solution. In the cold damp bleach mentioned above, 30 the liquor ratio is about 0.5 to 1.5. In the hot bleach using circulating hydrogen peroxide solutions, the liquor ratio is about 1:4 to 1:8. In order to obtain full whites from gray goods by this hot treatment, the goods must be treated at least 35 twice with the hot circulating bleaching liquor and in many instances additional treatments are required. Although excellent whites are obtained by the hot procedure, the consumption of energy is relatively high.

40 The present invention provides a method for bleaching cellulose readily and expeditiously in equipment presently employed. The present invention also provides a method for the production of full whites with a minimum consumption of energy and with a minimum consumption of 45 bleaching ingredient.

In accordance with the procedure of the present invention, gray goods are first treated under 50 conditions of low liquor ratio with an alkaline hydrogen peroxide bleach. The goods are partially bleached by this procedure and the motes and shives partially bleached and loosened. The goods are then rinsed and finished off under conditions of prevailing high liquor ratio by treat- 55 ing the goods at an elevated temperature with

a hot alkaline peroxide bleaching solution. When finished the goods possess a full white, are free of motes and shives, and possess substantially their original tensile strength. Additionally, the peroxide consumption in the hot bleaching solution is relatively low due to the fact that the goods have been treated in the damp condition with a peroxide solution and many of the catalytic effects traceable to the cellulose have there been eliminated and their action upon the hot 10 peroxide solution reduced to a minimum.

In carrying out the initial bleaching step of the present invention, the gray or unboiled goods are treated with an alkaline solution of hydrogen peroxide at room or moderately warm temperature 15 under conditions of low liquor ratio. The goods are dampened by any conventional method, whereby the fabric or fiber, whether raw stock, yarn, woven or knitted goods, is thoroughly wet out, or saturated with the desired bleaching solution, 20 and contain about 50 to 150% of solution based on the weight of goods. This step will usually include saturation of the goods with bleaching solution, as, for instance, by immersion therein and elimination of the surplus bleaching solution above that necessary to saturate the same by any well known means, as, for instance, by squeezing or hydroextracting, or by any known device or method, or the goods are saturated by any other convenient method and then permitted 25 to stand in the dampened or saturated condition until the desired bleach is obtained. This desired bleached condition is obtained after a period of a few hours to about 16 hours or more depending upon the kind of bleaching solution used 30 and the kind of goods.

The composition of bath effective for bleaching cellulose fibers with a low liquor ratio contains an alkali in addition to water and hydrogen peroxide, or some material generating hydrogen peroxide. This alkali may include materials acting as stabilizers for the hydrogen peroxide solution and may include, among others, silicate of soda, phosphates, such as sodium pyrophosphate, trisodium phosphate, disodium phosphate, sodium bicarbonate, borax, and the like. It is preferred, however, to use the well-known alkaline substances employed in bleaching operations, namely, caustic soda, soda ash, and the like. The quantity of alkaline material used should be considerably in excess of that thought permissible in circulating solutions and the alkali, calculated as sodium hydroxide, should be between about 5 and 50 g per liter.

It will be understood of course that additional 55

426

being treated, bleach-  
ing out agents. Item may be included in the bath  
solvents of various kinds and wet-  
bleaching fibers or filaments of cellulose in the  
damp condition contains in one liter thereof:  
100-volume hydro-  
gen peroxide. 5

15 Caustic soda  
42° Bé. silicate of soda  
100-volume hydro-  
gen peroxide. 5

16 The goods are saturated with the bleaching solution, the excess of the solution being expressed or eliminated whereby the goods retained from 50 to 150% of their original weight, or this quantity of bleaching solution is incorporated in the 20 goods in any other fashion. The dampened goods are then permitted to stand in this saturated condition from about 2 to 16 hours. In order to obtain bleaching in this dampened condition, the goods may be stacked, piled or stored and 25 generally covered in order to prevent evaporation or local changes in the concentration of the bleaching solution and to permit the goods to bleach in the damp condition with a liquor ratio, that is, the ratio of weight of treating solution to 30 weight of goods being treated therewith, of about 0.5 to 1.5.

The temperature of the goods may be maintained at room temperature or at temperatures somewhat above room temperature and in general at temperatures below 125° F. It will be understood where the temperature is high, the time of bleaching will be correspondingly low and also where the concentration of peroxide is high, somewhat shorter times are required to obtain 40 the desired bleaching effect than are required with lower concentration of bleaching ingredient.

After the goods have stood in the damp condition for the desired period of time, they may be rinsed and transferred to kiers for treatment 45 under conditions of high liquor ratio. After transference to a suitable heating vessel or kier, the goods are subjected to the final bleaching operation which includes treatment of the goods at elevated temperatures with a hot alkaline 50 circulating peroxide bleaching solution. The quantity of solution with respect to the quantity of goods is relatively high and the liquor ratio should be maintained at from about 1:4 to 1:8. The alkaline peroxide bleaching solution is circulated over and through the goods in any desired fashion and by the employment of any conventional means and in general the goods will be piled in a conventional type of kier. The time of treatment will be from about one hour 55 to about 10 hours and the temperature of the circulating solution will be above about 140° F. and in general form about 160° F. to 180° F.

The alkaline peroxide bleach suitable for use in the hot treatment contains in one liter approximately 5 cc. silicate and 3.5 cc. 100-volume hydrogen peroxide. At the end of the hot treatment the goods are removed, rinsed and finished in the usual manner.

As an example of the advantage of the present invention, it may be mentioned that in the bleaching of certain types of colored yarn goods the goods are desized, washed, and then subjected to two or more bleaching operations in which about 1½% hydrogen peroxide 100-volume, based on the weight of the goods, is em-

ployed, making therefore, a total peroxide consumption of 3% where two hot peroxide bleaches are necessary to obtain the desired white. In some instances substantially the same white can be obtained in one operation by increasing the peroxide content in the bleaching solution to 3% 100-volume hydrogen peroxide, based on the weight of the goods, and by heating for a longer period of time.

In accordance with the present invention 10 goods of the same quality and whiteness can be produced by employing from one third to one half less hydrogen peroxide. Not more than one half of the total hydrogen peroxide found necessary to obtain the desired bleach is incorporated 15 in the solution used for bleaching with a low liquor ratio, the remainder, of course, being incorporated in the bleaching solution used for bleaching with a high liquor ratio. In most instances it will be found expedient to incorporate 20 about 25 to 33% of the total peroxide in the first or low liquor ratio treatment and the remainder in the final bleaching step using a high liquor ratio.

In bleaching certain types of goods where two 25 hot hydrogen peroxide bleach baths are normally used (with the high liquor ratio), the present invention makes it possible to use considerably less peroxide by applying only one high liquor ratio treatment and one low liquor ratio 30 treatment. The low liquor ratio treatment may replace the entire desizing operation and thereby also eliminate one boil. In case only one boil is used with the regular operation, the time of this boil may be considerably shortened 35 by applying a cold low liquor ratio step first. Therefore in the treatment of goods requiring about 3% 100-volume hydrogen peroxide, based on the weight of the goods, the present invention makes possible the obtaining of goods of 40 equal white and quality by employing approximately 2% hydrogen peroxide, based on the weight of the goods, and in addition gives increased kier capacity with some saving in energy.

Another example is the bleaching of heavy goods, for instance, sheeting. Sheets are usually treated first with one alkali pressure boil or a plurality of alkaline open boils, followed by a bleaching treatment. In most cases the gray 50 goods are first subjected to a desizing operation, followed by a thorough wash. In accordance with the present invention the goods may be bleached to the same degree of white and to a better quality by subjecting the gray goods first to a low liquor ratio treatment, such as described, using approximately one third of the total amount of peroxide for bleaching. Thereafter the goods are washed and given a single 55 alkaline open boil treatment, followed by a hydrogen peroxide bleach using two thirds of the total amount, that is to say, the quantity of peroxide in the low liquor ratio treatment is about ½% of 100-volume hydrogen peroxide, based on the weight of the goods, and in the second approximately 1% 100-volume hydrogen peroxide, based on the weight of the goods. To bleach this type of sheeting according to the conventional method it would require over 2% 60 of hydrogen peroxide 100-volume.

The present invention therefore includes also a method to eliminate any desizing operation which is usually necessary before the goods are bleached to a full white or in all the cases where goods are later on dyed, printed, or fin- 75

111

2,231,426

3

ished, whereby residual impurities, especially starch, may cause difficulties or unevenness.

Although hydrogen peroxide has been described as the preferred bleaching agent, it will be under-

5 stood that materials generating hydrogen peroxide may be employed and to this end alkali metal and alkaline earth metal peroxides are suitable as are the perborates, percarbonates, per-phosphates, persilicates, and the like. These ma-  
10 terials, including hydrogen peroxide, being design-  
ated herein as peroxides.

It will be understood that the term "liquor ratio" refers to the relation between the weight of treating solution and the weight of goods  
15 treated therewith and that a low liquor ratio is one less than about 1.5 while a high liquor ratio is above about 4. The former is generally used in padding operations and the latter in circulat-  
ing operations.

20 1 claim:

1. A method for bleaching goods made of un-  
boiled cellulose which comprises treating the  
25 goods with an alkaline peroxide solution under  
conditions of low liquor ratio until a partial  
bleach is obtained and thereafter with an alkaline  
peroxide solution under conditions of high liquor  
ratio until a complete bleach is obtained.

2. A method for bleaching goods made of un-  
boiled cellulose which comprises treating the  
30 goods with an alkaline peroxide solution under  
conditions of low liquor ratio until a partial  
bleach is obtained and thereafter with an alkaline  
peroxide solution under conditions of high liquor  
35 ratio until a complete bleach is obtained, the al-  
kali concentration calculated as sodium hydroxide  
being higher in the first than in the second solu-  
tion.

3. A method for bleaching goods made of un-  
boiled cellulose which comprises treating the  
40 goods with an alkaline peroxide solution under  
conditions of low liquor ratio until a partial  
bleach is obtained and thereafter with an alkaline  
peroxide solution under conditions of high liquor  
45 ratio until a complete bleach is obtained, the tem-  
perature of treatment being lower in the first  
than in the second peroxide treatment.

4. A method for bleaching goods made of un-  
boiled cellulose which comprises incorporating in  
50 the goods from 50% to 150% of an alkaline per-  
oxide bleaching solution based upon the weight of  
the goods and then permitting the goods to stand  
and partially bleach, thereafter heating the goods  
55 in an alkaline peroxide solution under conditions  
of high liquor ratio and circulating the solution  
over and through the goods until a complete  
bleach is obtained.

5. A method for bleaching goods made of un-  
boiled cellulose which comprises incorporating in

the goods from 50% to 150% of an alkaline peroxide bleaching solution based upon the weight of the goods and then permitting the goods to stand and bleach at a temperature below 125° F., thereafter heating the goods in an alkaline peroxide solution at a temperature above 125° F. under conditions of high liquor ratio and circulating the solution over and through the goods until a complete bleach is obtained.

6. A method for bleaching goods made of un-  
boiled cellulose comprising incorporating in the  
10 goods more than 50% and less than 150% of an  
alkaline peroxide bleaching solution based upon  
the weight of the goods for partially bleaching  
the goods, and thereafter treating the goods under  
15 conditions of high liquor ratio with a hot cir-  
culating alkaline peroxide bleaching solution  
until a complete bleach is obtained.

7. A method for bleaching heavy goods, such  
as sheeting and the like, made of unboiled cellu-  
20 lose comprising incorporating in the goods more  
than 50% and less than 150% of an alkaline peroxide  
bleaching solution based upon the weight of the  
goods for partially bleaching the goods, then  
25 washing the goods and subjecting them to an  
alkaline boil and thereafter heating the goods  
under conditions of high liquor ratio in a hot  
circulating alkaline peroxide bleaching solution  
until a complete bleach is obtained.

8. A method for bleaching heavy goods, such as  
sheeting and the like, made of unboiled cellulose  
30 comprising incorporating in the goods more than  
50% and less than 150% of an alkaline peroxide  
bleaching solution based upon the weight of the  
goods for partially bleaching the goods, then  
35 washing the goods and subjecting them to an  
alkaline boil and thereafter heating the goods  
under conditions of high liquor ratio in a hot  
circulating alkaline peroxide bleaching solution  
until a complete bleach is obtained, the amount  
40 of peroxide employed in the second bleaching  
solution being about twice that in the first solu-  
tion.

9. A method for bleaching heavy goods, such  
as sheeting and the like, made of unboiled cellu-  
45 lose comprising incorporating in the goods less  
than 150% of an alkaline peroxide solution con-  
taining about  $\frac{1}{2}\%$  of peroxide calculated at 100  
volume hydrogen peroxide for partially bleaching  
the goods, then washing the goods and subject-  
50 ing them to an alkaline boil and thereafter heat-  
ing the goods under conditions of high liquor  
ratio in a hot circulating alkaline peroxide  
bleaching solution containing about 1% of per-  
oxide calculated as 100 volume hydrogen per-  
55 oxide until a complete bleach is obtained.

HANS O. KAUFFMANN.

CERTIFICATE OF CORRECTION.

Patent No. 2,231,426.

February 11, 1941.

HANS O. KAUFFMANN.

It is hereby certified that error appears in the printed specification of the above numbered patent requiring correction as follows: Page 3, second column, line 48, claim 9, for the word "at" read --as--; and that the said Letters Patent should be read with this correction therein that the same may conform to the record of the case in the Patent Office.

Signed and sealed this 11th day of March, A. D. 1941.

Henry Van Arsdale,

(Seal)

Acting Commissioner of Patents.